

## UNITED STATES PATENT OFFICE

HAROLD ROBERT RAFTON, OF LAWRENCE, MASSACHUSETTS, ASSIGNOR TO RAFFOLD PROCESS CORPORATION, A CORPORATION OF MASSACHUSETTS

## METHOD OF SIZING CARBONATE FILLED PAPER

No Drawing.

Application filed September 5, 1928. Serial No. 304,173.

This invention relates to the manufacture of paper and more particularly to an improved method of sizing paper filled with carbonate filler.

5 A principal object of this invention is to provide a method of sizing paper filled with carbonate filler wherein paraffin is employed as the sizing agent, the paraffin being employed in the form of a substantially non-breakable emulsion, the disperse phase of such emulsion being concentrated by the mutual precipitation or flocculation of two suitable precipitating agents in the presence of the emulsion at the wet end of the paper

15 machine.

Other objects and advantages of this invention will become apparent during the course of the following description.

In my copending application Serial No. 20 304,170, filed Sept. 5, 1928, I have described a process of sizing carbonate filled paper wherein a substantially nonbreakable paraffin emulsion is employed as the sizing agent, the disperse phase of such emulsion being 25 concentrated by the mutual precipitation of two precipitating agents such as sodium resinate and alum at an early stage in the paper making process, and wherein the sizing effect of the sizing agent which is wholly 30 or in part deteriorated by the action of the carbonate filler employed is restored by the subsequent addition to the paper mix of a suitable sizing restoring agent, such as alum. I have now discovered that a certain satisfactory measure of success can be obtained by 35 omitting the addition of one of the mutual precipitating agents such as alum at an early stage of the process and adding it to the paper mix at the wet end of the paper machine.

40 In the preferred practice of my process I add to fibrous material in a beater, mixer, or similar device carbonate filler, a substantially nonbreakable paraffin emulsion and sodium resinate in a sufficient amount as indicated below. Other material such as coloring matter may be added to the mix if desired. The mix is then passed through the usual preliminary steps in the paper making process and at or subsequent to the point 45 where the mix is diluted prior to its passage

on to a web-forming device of a paper machine, a suitable amount of a mutual precipitating agent such as alum, preferably in solution, is added to the mix, preferably continuously. In other words, this material is 55 added to the mix at the wet end of the paper machine. This results in the concentration of the disperse phase of the paraffin emulsion and the affixing of such disperse phase to the fibers whereby, after the passage of the mix 60 through the usual felting and finishing steps, a high grade sized carbonate filled paper is produced.

The amount of sodium resinate I may use is that amount which by itself when precipitated with alum, in accordance with my copending application Serial No. 304,172, filed Sept. 5, 1928, would not be sufficient to size 65 the paper, but would produce a substantially unsized paper. Thus the precipitate produced by sodium resinate and alum does not in this case act as a sizing agent but as a concentrating agent. Of course I may, if I desire, use a greater quantity of sodium resinate, but it is to be pointed out that it is possible to secure satisfactory sizing by my process where there is not enough sodium resinate used to impart sizing of itself. 75

By the addition of one of the mutually precipitating materials, such as the alum, at 80 the wet end of the paper machine, the alum is thus added at a point where there will be a minimum of intimacy and time of contact of the constituents of the mix, before the paper web is formed. It is necessary as indicated 85 to add the alum at or subsequent to the point of dilution of the mix, as I have found that if it be added when the mix is in relatively concentrated condition and particularly when the relatively concentrated mix is subjected to agitation as is normal in stock chests, the sizing effect in the mix is very quickly deteriorated even to the point of complete destruction. The sizing effect even when the mix is in the diluted condition 90 is gradually deteriorated, but is substantially unaffected within the time limits that the mix is maintained in the dilute state in the usual paper-making procedure. Moreover, although agitation in the dilute 95 100

state hastens to a certain extent the deterioration of the sizing effect, the speed of deterioration is not nearly so pronounced as in the concentrated condition, and from a practical standpoint I have found that the agitation to which the diluted mix is subjected prior to delivery onto the web-forming device does not deteriorate the sizing effect to a substantial degree.

10 Of course the other mutually precipitating material, such as the sodium resinate, may be added at any point prior to web formation other than in the beater; even after the addition of the alum, but experiments do not indicate that any substantially better sizing effect is obtained thereby, although the tendency to foam may be somewhat lessened, and such addition therefore can be considered the substantial equivalent 20 of adding sodium resinate in the beater.

Similarly of course it is obvious that the substantially nonbreakable emulsion may be added at any point prior to web formation other than in the beater, even after the addition of the alum, and such addition therefore can be considered the substantial equivalent of adding the substantially nonbreakable emulsion in the beater, providing only of course that the substantially nonbreakable emulsion must be present at the time when the sodium resinate and alum mutually precipitate so that its disperse phase may be concentrated thereby as previously described herein.

35 The alum solution need not be added directly to the fibrous mix, but can be added to the fresh water or white water, e. g. tray water, with which the mix is diluted. If the alum be added to the tray water, only a brief 40 time interval should elapse before the so treated tray water is used for dilution.

Although substantially more foam is produced in the herein described process than in the process referred to in my copending application, (except possibly in that modification wherein sodium resinate would be added at the wet end of the paper machine after the alum addition), nevertheless the foam is altered in character by the alum before the mix is passed onto the web-forming device, so that what foam is not held back in the rifflers or the like is of such nature that it causes substantially no trouble during the formation of the web, and the paper produced by this process is of a satisfactory quality. Moreover inasmuch as the amount of alum used in the present process is less than that used in the process set forth in my copending application referred to above, the present process therefore results in a more economical operation.

The substantially nonbreakable paraffin emulsion herein described should not be confused with paraffin emulsions prepared by employing a saponaceous emulsifying agent.

Nor should the emulsion be confused with emulsions made with an insoluble emulsifying agent such as colloidal clay, such for example as emulsions produced from pitchy or bituminous materials such as tar or asphalt. These various types of emulsions referred to differ in many respects from my substantially nonbreakable paraffin emulsion and are not suitable for use in the practice of my process.

75 The paraffin emulsions which I have found to be substantially nonbreakable by any of the chemical or mechanical agencies ordinarily employed in paper making in the concentrations or intensities at which they are normally used may be made in a variety of ways, for instance, with gums such as gum ghatti or gum arabic. While dextrin of itself does not appear to be suitable as an emulsifying agent, particularly if the emulsion is to be stored for any appreciable time, it does however appear to be useful in connection with the gums mentioned above. As the gums are normally much more expensive than dextrin, the dextrin may thus be used in conjunction with the gums to produce in general a lower cost emulsion. I have tested several formulae involving the use of gums and dextrin which give emulsions of essentially the nature desired, and which appear to work satisfactorily for the purpose. However, the one which I prefer to use in practice and which I have found to work well on a practical scale, is an emulsion made of paraffin with gum ghatti and dextrin as emulsifying agents. In one such emulsion, for example, which proved satisfactory, I used by weight as follows:

15 parts paraffin, 1 part gum ghatti, 1 part dextrin, 83 parts water.

105 As stated above so far as I have been able to discover by experiment, the emulsions which I employ are not affected in any way by any of the chemicals with which they come in contact at the concentrations at which they are used in the paper making process, nor are they affected by any of the mechanical agencies with which they come in contact at the intensities at which they are normally employed in the paper making process.

110 The reason for this latter characteristic is probably that the particles in my emulsions are surrounded with a film which is one or more molecules in thickness and hence entirely of negligible thickness compared with any insoluble emulsifier film. Hence such films cannot be knocked off or ruptured by ordinary mechanical means, as the thickness of this film is of entirely different order of magnitude (smaller) than are the clearances which obtain in the paper making machinery.

115 Of course it is not necessary that the emulsifier I use be water soluble in the sense that sodium chloride, for instance, is soluble, as materials which are known in the art as be-

ing colloidally soluble, are also suitable. For example gum ghatti which is suitable for my use may be considered to be in a measure colloidally soluble. With emulsifiers of the type 5 I employ the condition of the layer surrounding the disperse phase is such that by mechanical action in the paper making process, this layer is not disrupted, and therefore, the emulsion remains substantially nonbreakable 10 as heretofore indicated.

It is to be understood that I do not confine myself to the materials indicated above as being suitable for my emulsion since now that the principle of the use of a substantially 15 nonbreakable paraffin emulsion which is capable of having its disperse phase concentrated has been established in the paper industry, doubtless other similar emulsions will be evolved. Nor do I confine myself to the 20 definite concentration of the paraffin in the emulsion nor to definite proportions of emulsifying agents to each other or to the paraffin, as these may be varied in considerable degree 25 without affecting the desirable qualities of the emulsion.

Emulsions of the character referred to may be made in a variety of ways, as for example, in a dispersion machine such as any of a number of colloid mills or homogenizers. A 30 suitable way is to melt the paraffin, dissolve the emulsifying agent or agents in water, heat the emulsifying agent solution above the melting point of the paraffin and then feed the melted paraffin and the heated solution of 35 emulsifying agents jointly to the emulsifying machine.

In regard to the paraffin used, it is to be understood that either low or high melting point material can be employed. The so-called 40 fully refined paraffin is entirely satisfactory since it does not impart objectionable color to white sheets. However, for purposes of economy, it is often desirable to use a less pure material such for example as the material which is commonly known to the trade 45 as semi-refined paraffin scale, containing approximately 1-2 per cent of oil and water as impurities, which material gives satisfactory results. Such material will perhaps in 50 certain cases have varying melting points, but one particular sample used, for example, had a melting point of approximately 115° F. (46° C.). Other even more impure paraffins may be used, especially if the color 55 (whiteness) requirements of the finished paper are not too exacting, or if papers, other than white, are to be made.

As heretofore stated, in the preferred practice of my process I add at the wet end of the paper machine to a mix containing fibrous material sodium resinate and a substantially nonbreakable paraffin emulsion of the character referred to, a material which will mutually precipitate or flocculate with the sodium resinate present in the mix. This results in

the concentration of the disperse phase of the paraffin emulsion whereby such disperse phase becomes attached to the fibers and does not filter off therefrom during the passage of the mix over the web-forming device of the paper machine. The mutual precipitation or flocculation described serves, as stated; as a means for concentrating the disperse phase of the emulsion without breaking the emulsion, the disperse phase in the meantime being maintained in emulsified condition, and substantially nonbreakable by chemical or mechanical means. This concentration of the disperse phase appears to produce a complex which experiments indicate to be an intermediate between a true emulsion and a resolved or broken emulsion. For example, the complex can be temporarily dispersed by mechanical means but not diluted in the true sense as in the case of true emulsions. However, the complex can in a sense be diluted by dissolving the precipitate of the mutually flocculating agents therein and reconverting to a true emulsion. Thus while it is clear that the complex is not a true emulsion it is on the other hand, not a resolved emulsion. For example, the paraffin is not present in the concentrate as individual unitary deposited particles of paraffin, but rather in emulsified form, each particle being surrounded by a layer or film of emulsifying agent which prevents the individual particles from having contact not only with other particles of paraffin, but also from having contact with either the alum-sodium resinate precipitate, or the fibres, or other constituents of the fibrous mix. The existence of the paraffin in emulsified form is thus continued throughout the entire wet end of the paper making process. It is associated with the solids in the paper mix but is not deposited as paraffin thereon.

An illustrative furnish which may be advantageously used in the practice of my invention is as follows:

#### Materials added in the beater

|                                                                              | Pounds |
|------------------------------------------------------------------------------|--------|
| Fibrous furnish (e. g. sulphite and soda pulps)                              | 1700   |
| Rosin (added in the form of sodium resinate)                                 | 10     |
| Paraffin (added in the form of substantially nonbreakable paraffin emulsion) | 30     |
| Calcium carbonate magnesium hydroxide (carbonate filler)                     | 300    |

#### Material added proportionately and continuously on dilution

|      | Pounds |
|------|--------|
| Alum | 65     |

Another illustrative furnish is as follows:

#### Material added in the beater

|                                                                                          | Pounds |
|------------------------------------------------------------------------------------------|--------|
| Fibrous furnish (e. g. approximately equal parts of sulphite, soda and old paper stocks) | 1530   |
| Rosin (added in the form of sodium resinate)                                             | 10     |
| Paraffin (added in the form of substantially nonbreakable paraffin emulsion)             | 30     |
| "Broke" (containing calcium carbonate magnesium hydroxide (carbonate filler))            | 170    |
| Calcium carbonate magnesium hydroxide (carbonate filler)                                 | 300    |

*Material added proportionately and continuously on dilution*

|      | Pounds |
|------|--------|
| Alum | 65     |

5 In the above formulæ, the weights of carbonate filler refer to the bone dry basis, the weights of all other ingredients being given on the air dry basis.

In either of the above furnishes starch may 10 be used. It may be conveniently added to the beater subsequent to the addition of the carbonate filler, or otherwise if desired. Suitable coloring matter may be added if desired.

The illustrative furnishes given above produce satisfactorily sized paper, and, as will be apparent, the sizing can be increased or decreased by varying the relative quantities of the materials used in the above formulæ. The resultant paper may be used for such purposes as those to which sized papers are normally put including that as a raw stock for further conversion as for example for coating.

In place of alum in the practice of my 25 process I may employ with a measure of success an acid such as sulfuric acid ( $H_2SO_4$ ), an acid salt such as sodium bisulfate ( $NaHSO_4$ ), or a salt of a trivalent metal, such as ferric iron, or the other salts of aluminum. Of the aluminum salts available I may 30 use the chloride or the like, but I prefer to use ordinary "alum".

In place of sodium resinate I may use satisfactorily in the practice of my process other soaps, such as the oleates, or any partially or completely saponified material, such as saponified beeswax.

By the term "carbonate filler" as employed herein, is intended to be included calcium carbonate, of which lime mud from the causticizing process is one form; calcium carbonate magnesium basic carbonate employed in the paper disclosed in my U. S. Patent No. 1,595,416; calcium carbonate magnesium hydroxide disclosed in my U. S. Patent No. 1,415,391; or other substantially water insoluble normal or basic carbonates of alkaline earth metals, (which expression is herein intended to include magnesium), or compounds, 45 double salts, or physically associated mixtures of these with one or more other acid soluble materials of a substantially water insoluble nature. The term "carbonate filler" is also intended to include fibrous material 50 and/or other material such as paper coating constituents or the like containing one or more compounds of the character referred to, such as "old papers" or similar papers, "broke," or the like.

55 By the term "wet end of the paper machine" is intended to be included those instrumentalities employed in paper manufacture by which and/or in which a relatively concentrated paper mix is diluted, and treated, conveyed or fed up to the point of web-forma-

tion, such as the mixing box, regulating and proportioning devices, rifflers, troughs, screens, head boxes, inlets, and the like, including also instrumentalities used in the white water cycle.

When I employ the term "paraffin" herein, I mean paraffin wax, which is solid at ordinary or room temperature. I do not mean to restrict myself only to the paraffin hydrocarbons, but mean to include in this term 75 all the hydrocarbons of a waxy nature substantially unsaponifiable and inert to acidic and alkaline materials under ordinary conditions of temperature and pressure, whether derived from petroleum, shale, lignite, earth wax, or other natural or artificial sources. I do not, however, mean to include in this term material of a pitchy nature, such as bitumen or asphalt.

Where I use the term "sodium resinate" it 85 is to be understood that I mean it to include any material produced by the action of alkali, generally in aqueous solution, on rosin, or on natural or synthetic resin acid or acids, regardless of the exact composition of the 90 product, or the varying composition which different samples may possess.

When I use the word "paper" herein, I use it in the broad sense to include products of manufacture of all types and of all weights 95 and thicknesses, which contain as an essential constituent a considerable amount of prepared fiber and which are capable of being produced on a Fourdrinier, cylinder, or other forming, felting, shaping or molding machine.

100 While I have described in detail the preferred embodiment of my invention, it is to be understood that the details of procedure, the proportions of ingredients, and the arrangement of steps may be widely varied without departing from the spirit of the invention or the scope of the subjoined claims.

I claim:

1. The method of manufacturing a sized 110 paper filled with carbonate filler comprising adding to fibrous material a substantially nonbreakable paraffin emulsion and a substance which will react with a second substance subsequently to be added to form a 115 precipitate, said reaction serving to concentrate the disperse phase of said paraffin emulsion but not to break said emulsion, adding carbonate filler, thereafter adding said second precipitating substance under conditions 120 favoring the minimizing of the time of contact of the constituents of the mix, and thereafter making paper therefrom.

2. The method of manufacturing a sized 125 paper filled with carbonate filler comprising adding to fibrous material a substantially nonbreakable paraffin emulsion and a substance capable of reacting with a second substance subsequently to be added to form a 130

precipitate upon the fibrous material, said reaction serving to concentrate in association with said precipitate the disperse phase of said paraffin emulsion but not to break said emulsion, said precipitate being substantially incapable of having the paraffin associated therewith released from emulsified condition by mechanical means, adding carbonate filler, thereafter adding said second precipitating substance under conditions favoring the minimizing of the time of contact of the constituents of the mix, and thereafter making paper therefrom.

3. The method of manufacturing a sized paper filled with carbonate filler comprising adding to fibrous material a substantially nonbreakable paraffin emulsion and a substance which will react with a salt of a trivalent metal to form a precipitate, said reaction serving to concentrate the disperse phase of said paraffin emulsion but not to break said emulsion, adding carbonate filler, thereafter adding said salt of a trivalent metal under conditions favoring the minimizing of the time of contact of the constituents of the mix, and thereafter making paper therefrom.

4. The method of manufacturing a sized paper filled with carbonate filler comprising adding to fibrous material a substantially nonbreakable paraffin emulsion and a substance which will react with a salt of aluminum to form a precipitate, said reaction serving to concentrate the disperse phase of said paraffin emulsion but not to break said emulsion, adding carbonate filler, thereafter adding said salt of aluminum under conditions favoring the minimizing of the time of contact of the constituents of the mix, and thereafter making paper therefrom.

5. The method of manufacturing a sized paper filled with carbonate filler comprising adding to fibrous material a substantially nonbreakable paraffin emulsion and a substance which will react with alum to form a precipitate, said reaction serving to concentrate the disperse phase of said paraffin emulsion but not to break said emulsion, adding carbonate filler, thereafter adding said alum under conditions favoring the minimizing of the time of contact of the constituents of the mix, and thereafter making paper therefrom.

6. The method of manufacturing a sized paper filled with carbonate filler comprising adding to fibrous material a substantially nonbreakable paraffin emulsion and a substance which will react with a second substance subsequently to be added to form a precipitate, said reaction serving to concentrate the disperse phase of said paraffin emulsion but not to break said emulsion, adding carbonate filler, thereafter adding said second precipitating substance under conditions favoring the minimizing of the time and intimacy of contact of the constituents of the

mix, and thereafter making paper therefrom.

7. The method of manufacturing a sized paper filled with carbonate filler comprising adding to fibrous material a substantially nonbreakable paraffin emulsion and a substance which will react with a second substance subsequently to be added to form a precipitate, said reaction serving to concentrate the disperse phase of said paraffin emulsion but not to break said emulsion, adding carbonate filler, thereafter adding said second precipitating substance at the wet end of the paper machine, and thereafter making paper therefrom.

8. The method of manufacturing a sized paper filled with carbonate filler comprising adding to fibrous material a substantially nonbreakable paraffin emulsion and a substance which will react with a second substance subsequently to be added to form a precipitate, said reaction serving to concentrate the disperse phase of said paraffin emulsion but not to break said emulsion, adding carbonate filler, thereafter adding said second precipitating substance at a point in the process at which the mix is diluted preparatory to use on a web-forming device, and thereafter making paper therefrom.

9. The method of manufacturing a sized paper filled with carbonate filler comprising mixing with fibrous material a substantially nonbreakable paraffin emulsion, saponified material, and carbonate filler, thereafter adding a precipitant for said saponified material under conditions favoring the minimizing of the time of contact of the constituents of the mix, and thereafter passing the mix on to a web-forming device.

10. The method of manufacturing a sized paper filled with carbonate filler comprising mixing with fibrous material a substantially nonbreakable paraffin emulsion, saponified material, and carbonate filler, thereafter adding a precipitant for said saponified material at the wet end of the paper machine, and thereafter making paper therefrom.

11. The method of manufacturing a sized paper filled with carbonate filler comprising mixing with fibrous material a substantially nonbreakable paraffin emulsion, saponified material, and carbonate filler, thereafter adding alum at the wet end of the paper machine, and thereafter making paper therefrom.

12. The method of manufacturing a sized paper filled with carbonate filler comprising mixing with fibrous material a substantially nonbreakable paraffin emulsion, soap, and carbonate filler, thereafter adding alum at the wet end of the paper machine, and thereafter making paper therefrom.

13. The method of manufacturing a sized paper filled with carbonate filler comprising mixing with fibrous material a substantially nonbreakable paraffin emulsion, sodium resinate, and carbonate filler, thereafter adding

alum at the wet end of the paper machine, and thereafter making paper therefrom.

14. The method of manufacturing a sized paper filled with carbonate filler comprising mixing with fibrous material a substantially nonbreakable paraffin emulsion, sodium resinate, and carbonate filler, thereafter adding a precipitant for said sodium resinate at the wet end of the paper machine, and thereafter making paper therefrom.

15. The method of manufacturing sized paper filled with carbonate filler comprising mixing with fibrous material a substantially nonbreakable paraffin emulsion, sodium resinate in an amount insufficient of itself to impart a substantial degree of sizing to the paper, and carbonate filler, thereafter adding alum at the wet end of the paper machine, and thereafter making paper therefrom.

16. The method of manufacturing a sized paper filled with carbonate filler comprising mixing with fibrous material a paraffin emulsion made with gum ghatti as emulsifying agent, sodium resinate, and carbonate filler, thereafter adding alum at the wet end of the paper machine, and thereafter making paper therefrom.

17. The method of manufacturing a sized paper filled with carbonate filler comprising mixing with fibrous material a paraffin emulsion made with gum ghatti and dextrin as emulsifying agents, sodium resinate, and carbonate filler, thereafter adding alum at the wet end of the paper machine, and thereafter making paper therefrom.

18. In a method of manufacturing a sized paper filled with carbonate filler, the step of adding at the wet end of the paper machine a precipitant to a paper mix containing fibrous material, carbonate filler, a substantially nonbreakable paraffin emulsion and saponified material.

19. In a method of manufacturing a sized paper filled with carbonate filler, the step of adding at the wet end of the paper machine, a salt of a trivalent metal to a paper mix containing fibrous material, carbonate filler, a substantially nonbreakable paraffin emulsion and saponified material.

20. In a method of manufacturing a sized paper filled with carbonate filler, the step of adding at the wet end of the paper machine a salt of aluminum to a paper mix containing fibrous material, carbonate filler, a substantially nonbreakable paraffin emulsion and saponified material.

21. In a method of manufacturing a sized paper filled with carbonate filler, the step of adding at the wet end of the paper machine alum to a paper mix containing fibrous material, carbonate filler, a substantially nonbreakable paraffin emulsion and saponified material.

22. In a method of manufacturing a sized

paper filled with carbonate filler, the step of adding at the wet end of the paper machine alum to a paper mix containing fibrous material, carbonate filler, a substantially nonbreakable paraffin emulsion and soap.

23. In a method of manufacturing a sized paper filled with carbonate filler, the step of adding at the wet end of the paper machine alum to a paper mix containing fibrous material, carbonate filler, a substantially nonbreakable paraffin emulsion and sodium resinate.

24. That step in the method of manufacturing a sized paper filled with carbonate filler in which a paraffin emulsion is employed, comprising the addition of a precipitating substance to the paper mix at the wet end of the paper machine.

25. That step in the method of manufacturing a sized paper filled with carbonate filler in which a paraffin emulsion is employed, comprising the addition of acidic material to the paper mix at the wet end of the paper machine.

26. That step in the method of manufacturing a sized paper filled with carbonate filler in which a paraffin emulsion is employed, comprising the addition of metallic salt to the paper mix at the wet end of the paper machine.

27. That step in the method of manufacturing a sized paper filled with carbonate filler in which a paraffin emulsion is employed, comprising the addition of aluminum compound to the paper mix at the wet end of the paper machine.

28. That step in the method of manufacturing a sized paper filled with carbonate filler in which a paraffin emulsion is employed, comprising the addition of alum to the paper mix at the wet end of the paper machine.

In testimony whereof I affix my signature.

HAROLD ROBERT RAFTON.

110

115

120

125

130